

# United States Patent [19]

Hinoda et al.

[11]

4,432,844

[45]

Feb. 21, 1984

[54] **PROCESS FOR REGENERATION OF ELECTROLYTE CONTAINING TIN SALTS BY REDUCING THE SAME**

[75] Inventors: **Yuji Hinoda; Kazuhiro Enmoto**, both of Kawasaki, Japan

[73] Assignee: **Fujisash Company**, Kawasaki, Japan

[21] Appl. No.: **348,050**

[22] PCT Filed: **Jun. 23, 1980**

[86] PCT No.: **PCT/JP80/00141**

§ 371 Date: **Jan. 28, 1982**

§ 102(e) Date: **Jan. 28, 1982**

[87] PCT Pub. No.: **WO82/00036**

PCT Pub. Date: **Jan. 7, 1982**

[51] Int. Cl.<sup>3</sup> ..... **C25D 21/18**

[52] U.S. Cl. ..... **204/54 R; 204/DIG. 13**

[58] Field of Search ..... **204/54 R, DIG. 13; 423/89, 98**

## [56] References Cited

### U.S. PATENT DOCUMENTS

4,181,580 1/1980 Kitayama et al. ..... 204/28

### FOREIGN PATENT DOCUMENTS

51-39542 4/1976 Japan ..... 204/54 R  
52-89536 7/1977 Japan .  
53-110928 9/1978 Japan ..... 204/DIG. 13

### OTHER PUBLICATIONS

S. Baier, *Electro-Tinning*, International Tin Research and Development Council, Middlesex, England, 1939 pp. 11-12.

Primary Examiner—G. L. Kaplan

Assistant Examiner—William Leader

Attorney, Agent, or Firm—Frishauf, Holtz, Goodman & Woodward

### [57] ABSTRACT

Process for reclaiming stannous ion by reducing the same in an electrolyte to stannic ion through a simple operation in a short period of time, which comprises the steps of preparing the electrolyte in an acidic range as required and then adding metallic tin to the electrolyte and heating the mixture to at least 80° C., in order to reduce the stannous ion oxidized in the electrolyte containing tin salt to obtain a stable electrolyte treated product. This process may be utilized particularly for effectively reducing and reclaiming an electrolyte which contains tin salt used for electrolytically coloring aluminum.

4 Claims, No Drawings

PROCESS FOR REGENERATION OF  
ELECTROLYTE CONTAINING TIN SALTS BY  
REDUCING THE SAME

TECHNICAL FIELD OF THE INVENTION

This invention relates to a process for the reduction regeneration of an electro-plating bath or a coloring electrolyte for aluminum and more particularly to a process for the regeneration of an electrolyte by reducing stannic ions in the electrolyte into stannous ions through the addition of metallic tin to the used or old electrolyte.

BACKGROUND OF THE INVENTION

A tin salt aqueous solution containing stannous ions ( $\text{Sn}^{2+}$ ) is generally used as an electrolyte containing tin ions. This aqueous solution containing stannous ions is very unstable since stannous ions are easily oxidized into stannic ions ( $\text{Sn}^{4+}$ ) by oxygen in the air or oxygen generated during electrolysis.

As such stannic ions form in the electrolyte, the concentration of stannous ions in the electrolyte decreases and the current efficiency of electrolysis is reduced. Furthermore, it gives rise to the serious problem that the stannic ions become insoluble substances such as stannic acid, etc. which are likely to become colloids and therefore great difficulty is encountered in removing such insoluble substances by filtration. These insoluble substances attach onto the surface of the product and cause pitting thereon.

Therefore, in order to obtain good quality products, it is essential to control the concentration of stannic ions in the electrolyte.

With regard to preventing insoluble precipitates from forming, it is effective to add a chelating agent to the electrolyte to dissolve  $\text{Sn}^{4+}$ . In this case, however,  $\text{Sn}^{4+}$  is accumulated in the electrolyte, leading to an increase in the concentration of  $\text{Sn}^{4+}$  and, as a result, electrolytic coloring or electro-plating tend to become difficult. Therefore, a tin salt aqueous solution in which the concentration of stannic ions has increased by oxidation has had to be abandoned.

The regeneration of the electrolyte by the reduction thereof has been effected. One of such regeneration methods is an electrolytic reduction method as described in Japanese Patent Publication No. 19856/1978. In accordance with this electrolytic reduction method of stannous ions and stannic ions which are present in the electrolyte, the stannous ions are first reduced into metallic tin and thereafter the stannic ions are reduced into metallic tin. Therefore, although this method is excellent, a very long processing time is required and equipment and operation costs are increased.

Additionally, as the regeneration method of an electrolyte, a method of reducing stannic ions into stannous ions by adding those metals which are baser than tin has been carried out. According to this method, however, since the added metal is present in the electrolyte as a metal ion, it may exert bad influences on electrolytic processing. It is, therefore, necessary to remove such metal ions, but the removal operation of the metal ions is very complicated. Thus this method is not preferred from practical and economic standpoints.

The inventors have studied to develop a method which removes the disadvantages in the prior art as described above and which permits the reduction of stannic ions by a simplified procedure in a short time

and the formation of a regenerated electrolyte having a stable composition. As a result, it has been found that when metallic tin is added as a reducing agent to the electrolyte, as necessary, after the pH of the electrolyte has been controlled to the acidic region, the metallic tin and stannic ions undergo the oxidation-reduction reaction, promptly both changing into stannous ions.

DISCLOSURE OF THE INVENTION

10 This invention provides a process for the regeneration of an electrolyte containing tin salts by reduction thereof which is characterized in that in regenerating the electrolyte by reducing stannic ions therein into stannous ions, metallic tin is added to the electrolyte as it is or after the pH of the electrolyte is controlled to the acidic region and the resulting electrolyte is heated.

15 In accordance with the process of this invention, the stannic ions in the electrolyte are regenerated into stannous ions. After the reaction is completed, the unreacted metallic tin is taken out of the electrolyte and, as necessary, additional processings such as adjustment in the concentrations of other components in the electrolyte, adjustment in pH, etc. are applied. The thus regenerated electrolyte can be re-used.

20 When the above processings are continuously carried out, the electrolyte can be repeatedly used by recycling. Furthermore, in accordance with the process of this invention, the processing can be continuously carried out and the processing time can be greatly shortened. For example, in the method as described in Japanese Patent Publication No. 19856/1978, the time required for the reduction of the stannic ions is 6 hours or more whereas in the process of this invention, it is 1 hour or less and usually sufficient to be about 30 minutes.

25 Additionally, equipment and operation costs can be lessened and the quality of the product obtained by using the regenerated electrolyte can be stabilized.

30 PREFERRED EMBODIMENTS OF THE  
INVENTION

The electrolyte for use in this invention is subject to no special limitations so long as it contains tin salts. In a fresh electrolyte, almost all of the tin ions are stannous ions and there are almost no stannic ions. As the electrolysis proceeds, the concentration of stannic ions increases whereas the concentration of stannous ions relatively decreases.

35 The process of this invention is applied to an electrolyte in which the concentration of stannic ions has increased to a certain extent, for example, the ratio of  $\text{Sn}^{4+}/\text{Sn}^{2+}$  has reached  $\frac{1}{2}$  or more. In general, the electrolyte contains a chelating agent in order to keep the stannous and stannic ions in the state that they are dissolved.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550

thereof. In the process of this invention, sulfuric acid is most preferable.

The pH of the electrolyte is usually controlled to 4 or less and preferably to the range of from 0.5 to 2. Where the pH is too low, the reduction rate of stannic ions is somewhat reduced although metallic tin is promptly dissolved. On the other hand, where the pH exceeds 4, metallic tin is less dissolved and the reduction does not proceed promptly.

Thereafter, metallic tin is added to the electrolyte of which the pH has been controlled to the acidic region and the resulting electrolyte is heated. In this case, it is preferred to add metallic tin having high activity. For example, those having large specific surface areas, such as fine powder, tin foils, sponges, etc. are preferably used.

Metallic tin having such a high specific surface area can be produced as follows:

An acidic solution (e.g., an electro-plating solution or a coloring electrolyte for aluminum) containing stannous ions and/or stannic ions is used as an electrolyte and a direct current is passed through the electrolyte with electrically conductive materials such as metal or carbon as anode and cathode whereby tin ions ( $\text{Sn}^{2+}$ ,  $\text{Sn}^{4+}$ ) are deposited as metallic tin on the cathode. The thus obtained metallic tin is in a sponge form, has a high specific surface area and can be easily separated from the cathode.

The amount of the metallic tin added to the electrolyte is not limited and can be suitably determined depending upon the concentration of stannic ions in the electrolyte, the required concentration of stannous ions, etc. In general, it should be about 1 to 10 time moles of the amount required entirely to reduce stannic ions in the electrolyte. Even if the metallic tin is excessively added, the unreacted metallic tin precipitates in the bottom of the reactor and can easily be separated. Therefore, it imposes no specific hindrance onto the electrolyte and the metallic tin so separated can be re-used as it is.

In the process of this invention, it is required to heat the electrolyte to which the metallic tin has been added. The addition of metallic tin causes the oxidation-reduction reaction as illustrated below wherein the metallic tin and stannic ions react with each other, both forming stannous ions.



Since the reaction is accelerated by heating, it is preferred from the standpoint of acceleration of reaction to heat the electrolyte. However, where the electrolyte may be deteriorated in quality at high temperatures, the electrolyte to which metallic tin is added should be processed at low temperatures. From such standpoint, the heating temperature is generally set in the range of from 80° C. to the boiling temperature of the electrolyte.

With regard to the heating time, it is sufficient that the reduction reaction proceeds to the desired extent. While the heating time cannot be determined unconditionally since it varies depending upon the shape and amount of the metallic tin to be added and other various conditions, it is usually sufficient to be 1 hour or less.

The following examples are given to illustrate this invention in greater detail. In these examples, the concentration of stannic sulfate is shown as a concentration converted to  $\text{SnSO}_4$ .

5

#### EXAMPLE 1

##### (1) Production of Metallic Tin

A direct current was passed through an old or used coloring electrolyte for aluminum consisting of 9.0 grams/liter of stannous sulfate, 11.1 grams/liter of stannic sulfate, 70 grams/liter of citric acid and 20 grams/liter of sulfuric acid and having a pH of 1.5 with tin and stainless steel as anode and cathode respectively to deposit sponge-like metallic tin on the cathode.

##### (2) Regeneration by Reducing

To an old or used coloring electrolyte for aluminum consisting of 4.0 grams/liter of stannous sulfate, 15.1 grams/liter of stannic sulfate, 30 grams/liter of tartaric acid, 30 grams/liter of nickel sulfate and 20 grams/liter of ammonium sulfate and having a pH of 7.5 was added 40 grams/liter of sulfuric acid to adjust the pH to 0.9. Thereafter, 18 grams/liter of the sponge-like metallic tin as obtained in (1) was added to the above electrolyte and the resulting mixture was heated for 20 minutes at 100° C. After heating, the obtained electrolyte contained 21.2 grams/liter of stannous sulfate and 0.7 gram/liter of stannic sulfate.

20

#### EXAMPLE 2

To an old or used neutral tin electro-plating solution consisting of 41 grams/liter of stannous sulfate, 89 grams/liter of stannic sulfate, 150 grams/liter of ammonium citrate and 100 grams/liter of ammonium sulfate and having a pH of 6.5 was added 60 grams/liter of sulfuric acid to adjust the pH to 0.7. Thereafter, 148 grams/liter of the sponge-like metallic tin as obtained in Example 1 was added to the plating solution and the resulting mixture was heated at 96° C. for 40 minutes. After heating, the obtained plating solution contained 222 grams/liter of stannous sulfate and 8 grams/liter of stannic sulfate.

30

#### EXAMPLE 3

To an old or used lustrous tin-cobalt electro-plating solution consisting of 10 grams/liter of stannous sulfate, 10 grams/liter of stannic sulfate, 50 grams/liter of cobalt sulfate and 200 grams/liter of sodium pyrophosphate was added 60 grams/liter of sulfuric acid. Thereafter, 10.7 grams/liter of the sponge-like metallic tin as obtained in Example 1 was added to the plating solution and the resulting mixture was heated at 100° C. for 10 minutes. After heating, the obtained plating solution contained 21 grams/liter of stannous sulfate and 4 grams/liter of stannic sulfate.

35

#### EXAMPLE 4

To an old or used coloring electrolyte for aluminum consisting of 9.0 grams/liter of stannous sulfate, 11 grams/liter of stannic sulfate, 70 grams/liter of citric acid and 20 grams/liter of sulfuric acid and having a pH of 1.5 was added 21.4 grams/liter of the sponge-like metallic tin as obtained in Example 1. The resulting mixture was heated at 98° C. for 10 minutes. After heating, the obtained electrolyte contained 30 grams/liter of stannous sulfate and 4 grams/liter of stannic sulfate.

45

50

#### EXAMPLE 5

The procedure of Example 4 was repeated except that 100 mesh powdery tin reagent on the market was used in place of the sponge-like metallic tin. After heating, the obtained electrolyte contained 11.5 grams/liter of stannous sulfate and 9 grams/liter of stannic sulfate.

60

65

## COMMERCIAL UTILIZATION

The process of this invention is greatly useful for the regeneration of an electro-plating bath or a coloring electrolyte for aluminum containing tin salts. 5

We claim:

1. A process for regenerating a stannous tin-containing electrolyte which contains stannic ions comprising if said electrolyte is not acidic, adding sufficient acid to said electrolyte so that the electrolyte becomes acidic; adding metallic tin having a high specific surface area selected from the group consisting of powdered

tin, thin foils of tin, and sponge-like tin to said electrolyte; and heating said electrolyte containing said added metallic tin to from 80° C. to the boiling temperature of said electrolyte whereby stannic ions are reduced to stannous ions and metallic tin is oxidized to stannous ions thereby regenerating the electrolyte.

2. The process of claim 1 wherein the electrolyte to which the metallic tin is added has a pH of 4 or less.
3. The process of claim 1 wherein the electrolyte to which the metallic tin is added has a pH of from 0.5 to 2.
4. The process of claim 3 wherein sulfuric acid is added to said electrolyte to adjust the pH to the range of from 0.5 to 2.

\* \* \* \* \*

20

25

30

35

40

45

50

55

60

65